

April 1, 1969

D. K. MEYER ET AL  
DEVELOPER COMPOSITIONS AND THEIR USE  
IN ELECTROLYTIC ELECTROPHOTOGRAPHY

3,436,321

Filed Sept. 13, 1966

Sheet 1 of 2

FIG. 1



FIG. 2



INVENTORS  
DONALD K. MEYER  
ROBERT F. COLES  
BY *Carpenter, Kimsey & Coulter*  
ATTORNEYS

April 1, 1969

D. K. MEYER ET AL  
DEVELOPER COMPOSITIONS AND THEIR USE  
IN ELECTROLYTIC ELECTROPHOTOGRAPHY

3,436,321

Filed Sept. 13, 1966

Sheet 2 of 2

FIG. 3



FIG. 4



INVENTORS  
DONALD K. MEYER  
ROBERT F. COLES  
BY *Carpenter, Kinney & Coulter*  
ATTORNEYS

## 1

3,436,321

## DEVELOPER COMPOSITIONS AND THEIR USE IN ELECTROLYTIC ELECTROPHOTOGRAPHY

Donald K. Meyer, West St. Paul, and Robert F. Coles, North St. Paul, Minn., assignors to Minnesota Mining and Manufacturing Company, St. Paul, Minn., a corporation of Delaware

Filed Sept. 13, 1966, Ser. No. 579,114

Int. Cl. G03g 9/00

U.S. Cl. 204—18

6 Claims

This invention relates to novel developer compositions for use in electrolytic electrophotography. In one aspect this invention relates to an aqueous composition containing two or more developer materials which can be electrodeposited simultaneously in a wide range of continuously variable color density without a change of hue.

In electrolytic electrophotography a photoconductive copysheet having a strongly photoconductive layer on an electrically conductive substrate may be exposed to a light image and then electrolytically developed with the electrically conductive substrate connected as one electrode, preferably the cathode, and with the surface of the photoconductive layer in contact with a suitable developer solution which will effect a color change on the light struck areas of the copysheet surface. Such a process is described in U.S. 3,010,883. Particularly preferred color developers, such as those described in U.S. 3,172,826 and 3,172,827, may be utilized in multiple step processes to provide full color, continuous tone prints. Although black can be produced by the successive electrodeposition of cyan, magenta and yellow dyes, it is frequently desirable to electrodeposit a separate black image in a single step, and this may be achieved by using a developer containing dispersed carbon particles or a developer containing a silver salt.

To obtain developer dyestuffs which have the desired light absorption characteristics can be extremely difficult or impractical. Although it is possible to mix dyestuffs to obtain a desired color, dyestuffs tend to electrodeposit at varying rates from such an admixture, producing an undesirable change of hue over the normal density range. If magenta, cyan and yellow dyestuffs are admixed to produce a black color, the problem of differing electrodeposition rates is even more acute. Indeed the electrodeposition characteristics of a dyestuff admixture is generally not predictable from the electrodeposition rates and D log E curves of the individual dyestuffs therein. As a result, a good continuous gray scale is usually obtained by methods other than by using a combination of three dyestuffs in a single developer solution. Unfortunately, satisfactory "black" dyestuffs capable of rendering a neutral gray scale have not been found.

It is accordingly an object of this invention to provide an electrolytic electrophotographic developer solution having two or more dyestuffs which can be simultaneously electrodeposited onto a photoconductive copysheet without a significant hue change over the density ranges used.

Still another object of this invention is to provide a multidyestuff electrolytic electrophotographic developer solution which can be used to electrodeposit a continuous gray scale of photographic quality.

A further object of this invention is to provide an electrolytic electrophotographic developer of a desired color by admixing two or more dyestuffs.

Most electrolytically useful colored dyestuffs vary widely in their rates of electrolytic deposition, depending on such factors as chemical structure, concentration, development voltage and current, etc. Even under a given set of conditions, because the rate of deposition varies with the exposure, the plot of density (D) and log exposure (log E) is not a straight line. As would therefore be ex-

## 2

pected, mixing developer dyestuffs generally results in images of varying hue and unpredictable quality.

In accordance with this invention it has been found that two or more dyestuffs may be electrolytically deposited from an admixture without the abovementioned disadvantages, even though the individual dyestuffs may differ widely in their D log E curves. This effect appears to be generally independent of the size of the molecule and the chemical structure of the chromophoric group. Such dyestuffs have the formula



wherein D is a chromogenic radical, R is an alkyl radical having from 6 to 12 carbon atoms, R' is methyl or ethyl, n is 2 or 3, m is 2 or 3 and p is 0 or 1, where the controlling solubility characteristics of said dyestuff is attributable to the recited polyamine group. The chromogenic radical D may contain solubilizing groups, such as sulfonic acid, provided the effect of the polyamine group on the solubility is substantially retained, and the dyestuff is not rendered soluble in alkaline media. Thus, the dyestuffs of this invention are soluble in acidic media, particularly at a pH below about 6, but are insoluble in alkaline media. The chromogenic radical D is preferably selected from the following classes: azo, anthraquinone, anthrapyridone, phthalocyanine, quinacridone, thioindigo and xanthene. Preferably, the recited polyamine radical is linked to the chromogenic nucleus through a methylene, polymethylene, carbonyl or sulfonyl bridging radical. Dyestuffs of this class have been disclosed in U.S. 3,172,827. Any two or more dyestuffs of the above formula may be used together in aqueous acidic media in the form of their amine salts. The relative concentration of the respective dyestuffs is not generally critical and the effect is observed with wide ratios of the dye components (e.g., 9/1 to 1/9 weight ratio of two dyestuffs in admixture), although optimum results (i.e., no significant change of color or hue in the toe or shoulder or intermediate portions of the D log E curve) may be obtained within certain concentration ratios of the specific dyestuffs used. The total dyestuffs concentration in the solution is generally in the range of 0.1 to 5% by weight.

To illustrate the invention a variety of representative dyestuffs within the above formula were mixed in a single aqueous acidic solution and electrolytically deposited by the following procedure. In all instances the dyestuffs were utilized in amine salt form and were at least partially soluble in the aqueous acidic media. Each dyestuff was used as a 1-weight percent solution in dilute acid (pH 3-5.5), as indicated in U.S. Patent No. 3,172,827. Equal amounts of the dye solutions were then mixed together to form a mixture which could be electrolytically plated onto panchromatically sensitized photoconductive copysheets to obtain a variation in color gradation without significant change of hue throughout the useful density range, frequently up to a density of 2.5. The photoconductive copysheets used contained photoconductive zinc oxide in a styrene-butadiene copolymeric binder (6/1 weight ratio of ZnO to binder). The sheets were exposed through a 0-3 neutral density wedge and were developed for one second at 50 volts D.C. with the copysheet connected as cathode, using an apparatus of the type described in U.S. 3,172,827. The developed copysheets were then washed with water and dried with an air jet. These sheets were coated with lacquer to protect the image and were then evaluated in a recording densitometer using red, green and blue filters successively. The curves were then examined to confirm the visual observation of the plated image and to establish the absence of any undesirable cross over points in the respective curves, an indication of nonuniform and variable plating.

As will be seen in the data in Table I the dyestuffs of this invention, though having widely diverse D log E curves when measured individually, electrodeposit uniformly without significant color change over the useful density range. Although the theoretical explanation for these phenomena is not fully understood, it appears that the polyamine substituents on the dyestuff primary controls the rate of electrodeposition when two or more of such dyestuffs are deposited from solution. The dyestuffs employed in the illustrative examples are as follows:



Table I shows the results obtained with various dyestuff combinations within the scope of this invention, following the abovementioned procedures. Results are evaluated as excellent, good, fair or poor, representing increasing evidence of undesirable color over the den-

sity scale. Examples 28 and 29 illustrate the poor results observed with representative conventional cationic dyestuffs.

TABLE I

| Example | Dyestuffs | Density scale |
|---------|-----------|---------------|
| 1       | 2, 3      | Excellent.    |
| 2       | 1, 7      | Do.           |
| 3       | 2, 7      | Do.           |
| 4       | 1, 8      | Do.           |
| 5       | 2, 8      | Do.           |
| 6       | 1, 9      | Good.         |
| 7       | 2, 9      | Excellent.    |
| 8       | 2, 10     | Do.           |
| 9       | 3, 10     | Do.           |
| 10      | 1, 11     | Do.           |
| 11      | 3, 11     | Do.           |
| 12      | 6, 11     | Do.           |
| 13      | 1, 12     | Do.           |
| 14      | 3, 12     | Do.           |
| 15      | 6, 12     | Good.         |
| 16      | 1, 13     | Do.           |
| 17      | 3, 13     | Excellent.    |
| 18      | 6, 13     | Do.           |
| 19      | 1, 14     | Do.           |
| 20      | 3, 14     | Fair.         |
| 21      | 6, 14     | Excellent.    |
| 22      | 1, 15     | Do.           |
| 23      | 3, 15     | Do.           |
| 24      | 6, 15     | Fair.         |
| 25      | 2, 16     | Good.         |
| 26      | 3, 16     | Do.           |
| 27      | 6, 16     | Fair.         |
| 28      | 17, 18    | Poor.         |
| 29      | 19, 20    | Do.           |

FIGURES 1-4 illustrate the unusually smooth absorption curves obtained with the combination of three representative dyestuffs of this invention and, for purposes of comparison, the absorption curves of the individual dyestuffs using a 0-3 neutral density wedge. FIGURE 1 is a plot of density versus relative log exposure for the blue absorption of 0.75 weight percent yellow dyestuff No. 2, for the green absorption of 0.75 weight percent magenta dyestuff No. 1, and for the red absorption of 0.5 weight percent cyan dyestuff No. 3. The exposure was approximately 5 seconds at 100 foot candles with a development time of .3 second and development voltage of 75 volts D.C., anode spacing  $\frac{1}{2}$ -inch from copysheet surface. FIGURE 2 shows a similar series of runs with the same dyestuff, using a development time of 1.2 seconds. From FIGURES 1 and 2 will be seen that the individual absorption characteristics of the three dyestuffs differ quite markedly. FIGURES 3 and 4 are plots of density versus relative log exposure for the same dyestuffs after electrodeposition from admixture, the dyes in FIGURES 3 and 4 being obtained with development times of .3 and 1.2 seconds, respectively. FIGURES 3 and 4 show the coincidence of the red, blue and green absorption curves for the three component dye mixture and verify the remark-

ably similar plating characteristics and resulting neutral rendition of the gray scale.

Various other embodiments of the present invention will be apparent to those skilled in the art without departing from the scope thereof.

5 The embodiments of the invention in which an exclusive property or privilege is claimed are defined as follows:

1. An electrolytic electrophotographic developer which comprises at least two dyestuffs of the formula:



wherein D is a chromogenic radical, R is an alkyl radical having from 6 to 12 carbon atoms, R' is methyl or ethyl, n is 2 or 3 and p is 0 or 1, which dyestuffs are soluble in water at a pH below about 6 and are insoluble at a pH above 7.

2. The developer of claim 1 wherein D is a chromogenic radical of the azo, anthraquinone, anthrapyridone, phthalocyanine, quinacridone, thioindigo or xanthene type.

3. The developer of claim 1 wherein said dyestuffs are in amine salt form.

4. The developer of claim 1 having a cyan, a magenta and a yellow dyestuff in a proportion sufficient to reproduce a gray scale in electrolytic electrophotographic development.

5. In an electrolytic electrophotographic process the improvement which comprises using a developer containing at least two dyestuffs of the formula



wherein D is a chromogenic radical, R is an alkyl radical having from 6 to 12 carbon atoms, R' is methyl or ethyl, n is 2 or 3 and p is 0 or 1, which dyestuffs are soluble in water at a pH below about 6 and are insoluble at a pH above 7.

6. The process of claim 5 in which said dyestuffs include a cyan dyestuff, a magenta dyestuff and a yellow dyestuff in a proportion sufficient to reproduce a gray scale in electrolytic electrophotographic development.

#### References Cited

##### UNITED STATES PATENTS

- 45 3,010,883 11/1961 Johnson et al. ----- 204-18  
 3,172,826 3/1965 Tulagin et al. ----- 204-18  
 3,172,827 3/1965 Tulagin et al. ----- 204-18

JOHN H. MACK, Primary Examiner.

T. TUFARIELLO, Assistant Examiner.

UNITED STATES PATENT OFFICE  
CERTIFICATE OF CORRECTION

Patent No. 3,436,321

April 1, 1969

Donald K. Meyer et al.

It is certified that error appears in the above identified patent and that said Letters Patent are hereby corrected as shown below:

Column 2, line 11, "D-[NH(CH<sub>2</sub>)<sub>n</sub>]<sub>p</sub>-NH-(CH<sub>2</sub>)<sub>m</sub>NH'<sub>2</sub>" should read -- D[NH(CH<sub>2</sub>)<sub>n</sub>]<sub>p</sub>-NR-(CH<sub>2</sub>)<sub>m</sub>NR'<sub>2</sub> --. Column 3, lines 19 to 30, that portion of the formula reading



should read



same column 3, lines 55 to 57, that portion of the formula reading

]<sub>2</sub>

should read

]<sub>2-4</sub>

Column 6, lines 13 and 34, "ethyl,", each occurrence, should read -- ethyl, m is 2 or 3, --.

Signed and sealed this 14th day of April 1970.

(SEAL)

Attest:

EDWARD M. FLETCHER, JR.  
Attesting Officer

WILLIAM E. SCHUYLER, JR.  
Commissioner of Patents